# EUROPEAN PATENT SPECIFICATION

(11) **EP 3 255 209 B1**
(45) Date of publication and mention of the grant of the patent: **29.04.2020**
(21) Application number: 17175375.9
(22) Date of filing: 09.06.2017
(51) Int. Cl.: E01C 5/12, E01C 11/22

(54) **METHOD FOR PRODUCING A MANUFACTURED ARTICLE FOR ROAD KERBS AND/OR EDGINGS**
VERFAHREN ZUR HERSTELLUNG VON ERZEUGNISSEN FÜR STRASSENBORDSTEINE UND/ODER RANDEINFASSUNGEN
PROCÉDÉ DE PRODUCTION D'ARTICLE MANUFACTURÉ POUR ROUTE ET/OU DE BORDURES DE TROTTOIR

(30) Priority: 09.06.2016 IT UA20164233
(43) Date of publication of application: 13.12.2017
(73) Proprietor: Dr. Arch. Amantia Claudio Srl, 39020 Marlengo (IT)
(72) Inventor: AMANTIA, Claudio Marcello, 39020 MARLENGO (IT)
(74) Representative: Zamprogno, Bruno

(56) References cited:
- DE-A1- 19 744 476
- FR-A1- 2 712 014
- US-A- 4 151 344

## Description

The present invention concerns a method for the production of an elastomeric asphalt manufactured article for road kerbs and/or edgings.

In particular, the present invention concerns the production of manufactured road articles produced by means of an elastomeric asphalt conglomerate, usable for the formation of kerbs and/or edgings for cycle paths, pavements, traffic islands, speed humps, roundabouts, road barriers or similar to which the following description will explicitly refer without loss of generality.

There is often the need to intervene on stretches of road in asphalt to create road barriers or kerbs that delimit roundabouts, for example at crossroads, or create edgings which delimit traffic islands or pavements, or similar road constructions.

The methods currently used to produce a road kerb, for example for the construction of a roundabout, generally entail: performing cutting operations on the road surface, excavating the cut portion of the road surface to remove the asphalt, thus obtaining a roadbed with predefined depth for the creation of a foundation, positioning formworks in the excavated roadbed, arranging a steel reinforcement in the formworks, pouring cement into the formworks thus burying the reinforcement and creating a reinforced concrete base and, after solidification of the reinforced concrete base, positioning prefabricated concrete manufactured articles to rest on the base, then rigidly connecting the supporting surface of each manufactured article to the base below via a layer of mortar.

The methods described above are particularly complex and costly, and take a long time to produce with obvious consequences in terms of safety and traffic circulation.

Furthermore, said methods have a considerable environmental impact both in the production phase, since they require an operation to dispose of the asphalt removed for preparation of the bed, and when demolition of the existing kerbs is required since it is necessary to separate the concrete from the steel, with all resulting disposal costs.

DE 197 44 476 discloses a method for forming asphalt paving blocks for paving roadways wherein the paving blocks are plastic-coated asphalt block-like elements; FR 2 712 014 A1 discloses a surfacing slab composed of solid granulates coated and thermoplastic binder.

The Applicant has therefore carried out an in-depth study with the objective of identifying a solution relative to a method for producing manufactured articles for road kerbs or edgings which overcomes the above drawbacks.

The object of the present invention is therefore to make available a solution that allows achievement of the above objective.

The object of the present invention is therefore to produce a manufactured article for road kerbs and provide a method for producing said manufactured article.

This object is achieved by a method for producing the manufactured article as defined in the attached claims.

The present invention will now be described with reference to the accompanying drawings, which illustrate a non-limiting embodiment example thereof in which:
- Figure 1 is a schematic perspective view of the manufactured road article;
- Figures 2 to 6 show schematically an equal number of operating phases of the method for producing the manufactured article;
- Figure 7 shows schematically an example of installation on an asphalt road surface of the manufactured article;
- Figure 8 shows a section view of a portion of kerb arranged to rest on the asphalt road surface comprising two adjacent manufactured articles.

With reference to Figure 1, the number 1 indicates overall a manufactured article 1 structured to be used for creating road kerbs and/or edgings 100 and/or similar structures/works.

In the example shown in Figure 1, the manufactured article 1 can have, for example, a substantially elongated parallelepipedal shape which extends along a longitudinal axis L and consists of an elastomeric asphalt conglomerate indicated in Figures 2 to 6 by CAE. It is understood that the shape and section of the manufactured article 1 depends on the shape and section respectively of the kerb or edging to be produced.

The elastomeric asphalt conglomerate forming the manufactured article 1 comprises a first material and a second material appropriately metered and mixed with each other by means of the method that will be described in detail below.

The first material is based on an asphalt conglomerate (indicated by CA in Figures 2 and 5), being constituted of recycled asphalt, while the second material (indicated by CE in Figures 2 and 5) is based on elastomeric material. The asphalt conglomerate corresponding to the recycled asphalt can be conveniently obtained by removing the upper layer of an asphalt road. The recycled asphalt used can comprise pieces commonly indicated as pieces of "crust asphalt", having dimensions varying between approximately 5 cm and 50 cm, or, if obtained by means of milling and therefore broken up, the asphalt can comprise pieces having reduced dimensions, for example between approximately 3 cm and 5 cm.

The asphalt conglomerate forming the first material can comprise: filler (limestone or basaltic rock or similar), sand, inert materials (rubble or similar) having a predefined granulometry, and bitumen composed in turn of natural or residual hydrocarbons deriving from distillation or refinement of petroleum. Preferably, the recycled asphalt comprises a percentage of bitumen between approximately 3% and approximately 6% of the weight of the asphalt, preferably approximately 4%.

According to the invention, the second material based on elastomeric material consists of an elastomeric bituminous material, preferably polymerized.

The elastomeric bituminous material can comprise bitumen mixed with a percentage of elastomeric material ranging between approximately 3% and approximately 6%, preferably approximately 5% of the weight of the bitumen.

The elastomeric bituminous material can comprise preferably, but not necessarily, in addition to the bitumen and to the elastomeric material, also a percentage of plastomer material between approximately 3% and approximately 5%, preferably 4% of the weight of the bitumen.

The Applicant has found that an elastomeric bituminous material mixable with the recycled asphalt for production of the manufactured article is an elasto-bituminous sealant or a bitumen-rubber mastic, generally used for sealing road cracks.

For example, a bitumen-rubber mastic can correspond to the product named Stratos ARS 3.I TMP (Art IARS 31) marketed by ISOLTEMA ® Stick and Seal characterized by: an elastic recovery of 85%, a hardness of 60 Index and a softening temperature higher than 125°C. As regards the elasto-bituminous sealant, it consists of petroleum bitumen asphalt and elastomers with high toughness and resistance, micronized mineral fillers and stable plasticizers which do not exude and do not migrate. For example, the elasto-bituminous sealant can correspond to the products named Intermastik-C or Interplast 1806 produced by Interchimica SRL, or the product HELAX 15-KTF produced by the company "Italiana Bitumi ed Affini SRL" and characterized by softening point ranging from 95° to 125° and elongation - test piece 3 mm thick - greater than 1200%.

Preferably, the weight percentage of the elastomeric bituminous material in the manufactured article 1 can be between approximately 6% and approximately 10%, preferably 8%.

With reference to Figures 2 to 6, the method for producing the manufactured article 1 will be described below.

In particular, with reference to Figure 2, the method preferably comprises the step of arranging a given amount of asphalt conglomerate, preferably recycled and crushed/broken up (in a solid state), i.e. reduced to small pieces, obtained for example by means of milling and/or removal of the layer of asphalt forming the "crust" of a road surface.

The method further comprises the step of arranging a given amount of elastomeric bituminous material. The elastomeric bituminous material can preferably be composed of cakes preferably having a weight of approximately 10Kg or 25 Kg.

The method further comprises the step of arranging a melting-mixing system or apparatus 2, which is structured so as to: receive the first material, i.e. the asphalt conglomerate CA and the second material, i.e. the elastomeric bituminous material CE, heat the asphalt conglomerate CA and the elastomeric bituminous material CE thus bringing them to a liquid/semi-liquid state and mix the asphalt conglomerate CA and the elastomeric bituminous material CE thus forming an elastomeric asphalt conglomerate CAE which is homogeneous (without air bubbles) in the semi-liquid state.

According to an embodiment provided by way of example shown in Figure 2, the melting-mixing apparatus 2 can comprise a preferably cylindrical metal receptacle or container 3 adapted to receive and contain the asphalt conglomerate and the elastomeric bituminous material, heating equipment 7 adapted to heat the asphalt conglomerate CA and the elastomeric bituminous material CE under the control of the electronic control system 6, thus bringing both from a solid state to an approximately semi-liquid/liquid state, and mixing members 4 rotated inside the container 3 by a drive unit 5, preferably an electric motor controlled by an electronic control system 6, for mixing the asphalt conglomerate CA and the elastomeric bituminous material CE, thus obtaining the elastomeric asphalt conglomerate CAE in an approximately semi-liquid/liquid state.

The heating equipment 7 can comprise for example resistive electric elements and/or gas or diesel burners and/or pipes for the circulation of diathermic oil or similar devices adapted to provide heat preferably to the walls of the container 3.

With reference to Figure 3, the method further entails arranging at least one formwork or forming mould 8, preferably made of metallic material, which has an inner seat/cavity 9 that reproduces in negative the outer shape of the manufactured article 1 to be produced.

With reference to Figure 2, the method comprises the step of feeding/pouring the asphalt, preferably in fragments or crust, and the elastomeric bituminous material, preferably in the form of cakes, into the container 3.

It is understood that the quantity of asphalt conglomerate CA and the quantity of elastomeric bituminous material fed/poured into the container 3 depends on the number of manufactured articles 1 to be produced. If N manufactured articles have to be produced, a quantity of the first and second material is fed in, corresponding to the first and second quantity respectively, each multiplied by a multiplication factor N.

For example, if approximately 1500 Kg of elastomeric asphalt conglomerate CAE have to be produced to create a plurality of manufactured articles, approximately 90 Kg of cakes of elastomeric bituminous material and approximately 1410 Kg of recycled asphalt can be used, for example.

In the example shown and described in Figures 2-6 reference will be made, solely in order to increase understanding of the present invention, to the production of one single manufactured article 1.

With reference to Figure 2, the method comprises the step of controlling by means of the electronic control system 6 the heating equipment 7, to heat, for example by means of the walls of the container 3, the asphalt conglomerate CA constituting the first material and the elastomeric bituminous material CE constituting the second material, thus bringing them to a predefined melting temperature. The electronic control system 6 further controls rotation of the mixing members 4 for mixing the asphalt conglomerate CA and the elastomeric bituminous material CE, which have been melted, thus obtaining the homogeneous elastomeric asphalt conglomerate CAE.

Preferably, the heating equipment 7 is controlled so that the melting temperature is maintained between approximately 160°C and approximately 200°C, preferably 180°C, while the mixing range can be between approximately two hours and approximately six hours, preferably four hours.

The method further comprises the step of feeding/pouring the homogeneous elastomeric asphalt compound CAE present in the container 3 into the seat/cavity 9 of the mould 8 (Figure 5) . Preferably, before pouring the elastomeric asphalt conglomerate CAE into the seat/cavity 9 of the mould 8, the method comprises the step of depositing/covering the inner surface of the seat/cavity 9 by means of a release agent DIS (Figure 4) structured to detach the elastomeric asphalt compound CAE from the inner metallic surface of the seat/cavity 9 after solidification of the elastomeric asphalt compound CAE in the seat 9.

Preferably, the agent DIS is a silicone-based material. For example, a release agent can correspond to the product E 55 LO ® marketed by F.IN.CO S.R.L.

The method further comprises the step of cooling the elastomeric asphalt conglomerate CAE in the cavity 9 of the mould 8 for a predefined solidification period and at the end of the latter, extracting the solidified manufactured article 1 from the cavity 9 of the mould (Figure 6). Preferably the solidification period can range between approximately two four and approximately six hours.

The method can further comprise the step of carrying out a surface finishing operation on the outer surface of the manufactured article 1 thus making it coarse/rough so as to obtain a non-slip surface. The Applicant has found that a coarse/rough outer surface of the manufactured article conveniently increases the grip of the wheels which come into contact with the contact surface of the manufactured article, for example at roundabouts, and therefore reduces the risk of slipping/falling of motorcyclists. According to a possible embodiment, the surface finishing operation on the outer surface of the manufactured article 1 can be carried out by sandblasting. The sandblasting can be performed with a sandblaster generating an air mixture of compressed air and abrasive microspheres having dimensions ranging between approximately 0.5 mm and 2 mm, preferably between approximately 0.7 mm and approximately 1.2 mm.

The method can further comprise the step of superficially colouring the manufactured article 1 thus creating road markings in the form of lines/images. The Applicant has found that the asphalt composition of the manufactured article and the coarse/rough surface allow the use of coloured paints for asphalt. It should be specified that the paints applied on concrete manufactured articles (known art) form a surface film which tends to detach/deteriorate in a relatively short time, whereas the paints for asphalt when applied to the manufactured article produced according to the teachings of the present invention adhere and penetrate permanently therein for a certain depth. Therefore the use of paints for asphalt in the manufactured article described considerably prolongs the life of the marking lines/images. The paint for asphalt (RAL for asphalt) could be a solvent paint based on modified glycerophthalic resins and chlororubber and could comprise, for example, the paint named SPARTITRAFFICO produced by IVAS spa.

It is understood that the method allows the production of a plurality of manufactured articles and therefore entails a plurality of moulds 8 inside which the elastomeric asphalt conglomerate CAE can be poured.

According to the invention, the melting-mixing apparatus 2 can have a transportable structure and/or be self-propelled so that it can be conveniently positioned in the place in which the kerb or edging 100 is required. In this case, with reference to Figure 7, the method comprises the step of arranging moulds 8 shaped so as to allow production of the manufactured article directly on the surface S. For example, the moulds 8 can be shaped so as to allow injection from above of the elastomeric asphalt conglomerate CAE into the seat 9 and allow extraction of the manufactured article 1 by raising the mould 8 upwards, for example in a vertical direction. In this case, the method comprises the step of positioning the moulds 8 in the points/areas in which the manufactured articles are required so as to present, namely the opening of the mould 8 for extraction of the manufactured article 1 facing the asphalt surface S, injecting the elastomeric asphalt conglomerate CAE into the seats 9 of the moulds 8 so that the elastomeric asphalt conglomerate CAE is deposited on the surface of the asphalt S and, after the solidification period of the conglomerate inside the mould 8, sliding the mould 8 off the manufactured article 1 by vertically raising the mould 8 thus separating it from the manufactured article 1 which, during solidification, has become fixed to the surface S of the asphalt layer.

The applicant has found that in this way non-removable fixing is conveniently obtained between the lower base B of the manufactured article 1, which is in a semi-solid (softened) state, and the underlying asphalt road surface S. This is possible due to the fact that the asphalt composition of the manufactured article is substantially compatible with the composition of the asphalt of the road. In this way the manufactured article 1 is rigidly joined to the underlying road surface.

According to a possible example, which is not part of the present invention, in which the manufactured article 1 is prefabricated and transported to the place in which construction of the kerb is required, the method comprises, during installation of the manufactured article 1, the step of heating the base B of the solid manufactured article 1 thus bringing it to a semisolid softened state and laying the same on the underlying asphalt surface S so that the base B is fixed/joined in a non-removable manner to the surface S.

With reference to Figure 8, according to a possible example, which is not part of the present invention, in which the manufactured article is prefabricated and transported to the place where construction of the kerb 100 is required, the method comprises the step of joining/fixing the base B of the manufactured article 1 to the road surface S by means of the interposition of a tape/film R made of elastomeric bituminous material appropriately heated/softened.

The method has numerous advantages: the elastomeric asphalt composition of the manufactured article allows the latter to be installed directly on the upper part of the road surface in a simple rapid manner and at low cost.

Furthermore, the presence of the elastomeric component in the manufactured article allows the same to elastically withstand the mechanical stress generated on it during the passage of vehicles. Furthermore, the simplicity of execution of the method allows production of the manufactured article directly on the road construction site. Furthermore, the method allows the manufactured article to be produced from a recycled product, i.e. asphalt. Lastly, the manufactured article, due to its composition substantially similar to that of asphalt, can be demolished and recycled simultaneously with the demolition/reconstruction of an asphalt road surface with all the advantages this entails in environmental terms and in terms of containment of the demolition costs.

Lastly it is clear that modifications and variations as established by the claims can be made to the method without departing from the scope of the present invention.

## Claims

1. Method for producing an elastomeric asphalt manufactured article (1) for road kerbs and/or edgings (100) comprising the steps of:
arranging a given amount of asphalt conglomerate (CA) and a given amount of elastomeric material (CE) in a container (3),
said asphalt conglomerate (CA) being constituted of recycled asphalt,
said elastomeric material (CE) being constituted of elastomeric bituminous material comprising an elasto-bituminous sealant or a bitumen-rubber mastic,
heating said asphalt conglomerate (CA) and said elastomeric material (CE) in said container (3) so as to cause said asphalt conglomerate (CA) and said elastomeric material (CE) to change from a solid state to a semi-liquid/liquid state,
mixing said asphalt conglomerate (CA) and said semi-liquid/liquid elastomeric material (CE) so as to obtain a homogeneous elastomeric asphalt conglomerate (CAE) in a semi-liquid/liquid state,
pouring the homogeneous elastomeric asphalt conglomerate (CAE) in semi-liquid/liquid state into a cavity (9) of a forming mould (8) shaped so as to make a negative trace of the shape of the manufactured article (1) to produce,
extracting the manufactured article (1) from said cavity (9) of said mould (8) following a predetermined solidification period,
the method being characterised of:
arranging said mould (8) on the asphalt surface (S) on which the kerb or edging (100) is to be produced, wherein the opening of the mould (8) for extraction of the manufactured article 1 facing the asphalt surface (S),
pouring said elastomeric asphalt conglomerate (CAE) into the seat (9) of said mould (8) so that the elastomeric asphalt conglomerate (CAE) forming the supporting base (B) of the manufactured article (1) is deposited on, and solidifies in contact with, the asphalt surface (S) below,
raising the mould (8) upwards thus separating it from the manufactured article (1) which, during solidification, has become fixed to the surface (S) of the asphalt layer.

2. Method according to claim 1, wherein the elastomeric bituminous material (CE) comprises a percentage of elastomeric material from about 3% to about 6% by weight of the bitumen.

3. Method according to claim 1, wherein said step of pouring the semi-liquid/liquid homogeneous elastomeric asphalt conglomerate (CAE) into said cavity (9) of said mould (8) is preceded by the step of depositing on the internal surface of said cavity (9) a silicone-based release agent (DIS).

4. Method according to claim 1, comprising the step of heating said asphalt conglomerate (CA) and said elastomeric material (CE) so as to reach a melting temperature of 180° C, while the mixing range can be between approximately two hours and approximately six hours.

5. Method according to any of the foregoing claims, comprising carrying out a surface finishing operation on the outer surface of the manufactured article (1) thus making it coarse/rough so as to obtain a non-slip surface.

6. Method according to claim 5, wherein the surface finishing operation on the outer surface of the manufactured article (1) is carried out by sandblasting.

7. Method according to any of the foregoing claims, comprising superficially colouring the manufactured article (1) by coloured paints for asphalt in order to creating road markings in the form of lines/images.

8. Method according to any of the foregoing claims, comprising the step of arranging a given amount of asphalt conglomerate, recycled and crushed/broken up, reduced to small pieces, obtained by means of milling and/or removal of the layer of asphalt forming the crust of a road surface.

## Patentansprüche

1. Verfahren zur Herstellung eines aus elastomeren Asphalt hergestellten Erzeugnisses (1) für Straßenbordsteine und/oder Randeinfassungen (100), mit folgenden Schritten:
Anordnen einer bestimmten Menge Asphaltkonglomerats (CA) und einer bestimmten Menge Elastomermaterials (CE) in einem Behälter (3),
wobei das Asphaltkonglomerat (CA) aus recyceltem Asphalt besteht,
wobei das Elastomermaterial (CE) aus elastomerem bituminösem Material besteht, das ein elastomeres bituminöses Dichtungsmittel oder ein Bitumen-Gummi-Mastix aufweist,
Erhitzen des Asphaltkonglomerats (CA) und des Elastomermaterials (CE) in dem Behälter (3), um zu bewirken, dass das Asphaltkonglomerat (CA) und des Elastomermaterial (CE) aus einem Festzustand in einen halbflüssigen/flüssigen Zustand übergehen,
Mischen des Asphaltkonglomerats (CA) und des halbflüssigen/flüssigen Elastomermaterials (CE), um ein homogenes elastomeres Asphaltkonglomerat (CAE) in einem halbflüssigen/flüssigen Zustand zu erhalten,
Gießen des homogenen elastomeren Asphaltkonglomerats (CAE) in einem halbflüssigen/flüssigen Zustand in einen Hohlraum (9) einer Gussform (8), die derart geformt ist, dass eine negative Spur der Form des hergestellten Erzeugnisses (1) entsteht,
Extrahieren des hergestellten Erzeugnisses (1) aus dem Hohlraum (9) der Form (8) nach einer vorbestimmten Erstarrungszeit,
wobei das Verfahren durch Folgendes gekennzeichnet ist:
Anordnen der Form (8) auf der Asphaltoberfläche (S), auf welcher der Bordstein oder die Randeinfassung (100) hergestellt werden soll, wobei die Öffnung der Form (8) für die Extraktion des hergestellten Erzeugnisses (1) der Asphaltoberfläche (S) zugewandt ist,
Gießen des elastomeren Asphaltkonglomerats (CAE) in den Sitz (9) der Form (8), so dass das elastomere Asphaltkonglomerat (CAE), das die Trägerbasis (B) des hergestellten Erzeugnisses (1) bildet, auf der darunter befindlichen Asphaltoberfläche (S) abgesetzt wird und in Kontakt damit erstarrt,
Hochheben der Form (8), um diese somit von dem hergestellten Erzeugnis (1) zu trennen, welches während der Erstarrung an der Oberfläche (S) der Asphaltschicht fixiert wurde.

2. Verfahren nach Anspruch 1, wobei das elastomere bituminöse Material (CE) einen Gewichtsanteil an Elastomermaterial von etwa 3 % bis etwa 6 % des Bitumens aufweist.

3. Verfahren nach Anspruch 1, wobei vor dem Schritt des Gießens des halbflüssigen/flüssigen homogenen elastomeren Asphaltkonglomerats (CAE) in den Hohlraum (9) der Form (8) der Schritt des Aufbringens eines silikonbasierten Trennmittels (DIS) auf der Innenfläche des Hohlraums (9) erfolgt.

4. Verfahren nach Anspruch 1, mit dem Schritt des Erhitzens des Asphaltkonglomerats (CA) und des Elastomermaterials (CE) zum Erreichen einer Schmelztemperatur von 180 °C, während der Mischbereich zwischen etwa zwei Stunden und etwa sechs Stunden liegen kann.

5. Verfahren nach einem der vorstehenden Ansprüche, welches das Ausführen eines Oberflächenveredelungsvorgangs auf der Außenfläche des hergestellten Erzeugnisses (1) umfasst, wodurch das Erzeugnis (1) rau/uneben wird, um eine rutschfeste Oberfläche zu erhalten.

6. Verfahren nach Anspruch 5, wobei der Oberflächenveredelungsvorgang auf der Außenfläche des hergestellten Erzeugnisses (1) mittels Sandstrahlung durchgeführt wird.

7. Verfahren nach einem der vorstehenden Ansprüche, welches das Färben der Oberfläche des hergestellten Erzeugnisses (1) mittels eines farbigen Anstrichs für Asphalt umfasst, um Fahrbahnmarkierungen in der Form von Linien/Bildern zu erstellen.

8. Verfahren nach einem der vorstehenden Ansprüche, mit dem Schritt des Anordnens einer bestimmten Menge von Asphaltkonglomerat, das recycelt und zerschlagen/gebrochen wird, zu kleinen Stücken zerkleinert wird und durch Fräsen und/oder Entfernen der Asphaltschicht, welche die Kruste einer Fahrbahnoberfläche bildet, erhalten wird.

## Revendications

1. Procédé de production d'un article manufacturé en asphalte élastomère (1) pour des bordures de chaussée et/ou des bordures de trottoir (100) comprenant les étapes consistant à :
agencer une quantité donnée de conglomérat d'asphalte (CA) et une quantité donnée de matériau élastomère (CE) dans un contenant (3),
ledit conglomérat d'asphalte (CA) étant constitué d'asphalte recyclé,
ledit matériau élastomère (CE) étant constitué de matériau bitumeux élastomère comprenant un produit d'étanchéité élasto-bitumeux ou un mastic de bitume-caoutchouc,
chauffer ledit conglomérat d'asphalte (CA) et ledit matériau élastomère (CE) dans ledit contenant (3) de sorte à amener ledit conglomérat d'asphalte (CA) et ledit matériau élastomère (CE) à passer d'un état solide à un état semi-liquide/liquide,
mélanger ledit conglomérat d'asphalte (CA) et ledit matériau élastomère semi-liquide/liquide (CE) de sorte à obtenir un conglomérat d'asphalte élastomère homogène (CAE) dans un état semi-liquide/liquide,
verser ledit conglomérat d'asphalte élastomère homogène (CAE) à l'état semi-liquide/liquide dans une cavité (9) d'un moule de formage (8) façonné de sorte à décrire un négatif de la forme de l'article manufacturé (1) à produire,
extraire l'article manufacturé (1) de ladite cavité (9) dudit moule (8) après une période de solidification prédéterminée,
le procédé étant **caractérisé par** le fait de :
agencer ledit moule (8) sur la surface d'asphalte (S) sur laquelle la bordure de chaussée ou bordure de trottoir (100) doit être produite, où l'ouverture du moule (8) destinée à l'extraction de l'article manufacturé (1) fait face à la surface d'asphalte (S),
verser ledit conglomérat d'asphalte élastomère (CAE) dans la cavité (9) dudit moule (8) de sorte que le conglomérat d'asphalte élastomère (CAE) formant la base de support (B) de l'article manufacturé (1) est déposé sur, et se solidifie au contact de, la surface d'asphalte (S) se trouvant en dessous,
soulever le moule (8) vers le haut en le séparant ainsi de l'article manufacturé (1) lequel, lors de la solidification, a adhéré à la surface (S) de la couche d'asphalte.

2. Procédé selon la revendication 1, dans lequel le matériau bitumeux élastomère (CE) comprend un pourcentage de matériau élastomère allant d'environ 3 % à environ 6 % en poids du bitume.

3. Procédé selon la revendication 1, dans lequel ladite étape consistant à verser le conglomérat d'asphalte élastomère homogène semi-liquide/liquide (CAE) dans ladite cavité (9) dudit moule (8) est précédée par l'étape consistant à déposer sur la surface interne de ladite cavité (9) un agent de démoulage à base de silicone (DIS).

4. Procédé selon la revendication 1, comprenant l'étape consistant à chauffer ledit conglomérat d'asphalte (CA) et ledit matériau élastomère (CE) de sorte à atteindre une température de fusion de 180 °C, la période de mélange pouvant aller d'approximativement deux heures à approximativement six heures.

5. Procédé selon l'une quelconque des revendications précédentes, comprenant le fait de réaliser une opération de finition de surface sur la surface extérieure de l'article manufacturé (1) en la rendant ainsi plus grossière/rugueuse de sorte à obtenir une surface non glissante.

6. Procédé selon la revendication 5, dans lequel l'opération de finition de surface sur la surface extérieure de l'article manufacturé (1) est réalisée par sablage.

7. Procédé selon l'une quelconque des revendications précédentes, comprenant le fait de colorer superficiellement l'article manufacturé (1) au moyen de peintures de couleur destinées à l'asphalte de sorte à créer des marquages routiers sous la forme de lignes/d'images.

8. Procédé selon l'une quelconque des revendications précédentes, comprenant le fait d'agencer une quantité donnée de conglomérat d'asphalte, recyclé et broyé/concassé, réduit en petits morceaux, obtenu par fraisage et/ou retrait de la couche d'asphalte formant la croûte d'une surface de chaussée.
